

# United States Patent Office

3,166,507

Patented Jan. 19, 1965

1

3,166,507

## LUBRICATING OILS CONTAINING ALKYL ACRYLATE-VINYLPYRIDINE N-OXIDE COPOLYMERS

Frederick E. Bailey, Jr., Charleston, and Walter J. Toussaint, South Charleston, W. Va., assignors to Union Carbide Corporation, a corporation of New York

No Drawing. Filed Aug. 13, 1962, Ser. No. 216,348  
6 Claims. (Cl. 252—51.5)

This invention relates to novel compositions comprising lubricating oils containing polymerized compounds as viscosity index improvers and engine sludge dispersants. More particularly, this invention relates to novel copolymers comprising polymerized esters of acrylic acid and vinylpyridine N-oxides used in lubricating oils as additives and viscosity index improvers.

The art of adding additives to lubricating oil compositions adapted for use in internal combustion engines is well known to those versed in this field and has resulted in substantial improvements in lubricants. However, in view of the extent to which motor transport is a dominating feature of our existence, the search for useful additives for lubricating oil compositions is a never-ending one and hence this art is in a constant and necessary state of flux. It is with this art that this invention is primarily concerned.

The novel copolymers employed in this invention comprise as polymeric components thereof, a major amount of an ester of acrylic acid and an aliphatic alcohol containing up to 18 carbon atoms, and a minor amount of a vinylpyridine N-oxide or a lower-alkyl substituted vinylpyridine N-oxide.

As used throughout this specification, the term "lower-alkyl" relates to alkyl groups containing from one to six carbon atoms and in addition, the terms vinylpyridine N-oxide and lower-alkyl substituted vinylpyridine N-oxide include both the hydrated and anhydrous forms. The dihydrate form, being more stable, is preferred. As is known in the art, the hydrated form of an amine oxide is produced by simple addition of water, for example, merely by picking up moisture from the air.

As pointed out hereinabove, the novel copolymers employed as lubricating oil additives comprise a major amount of an ester of acrylic acid, and a minor amount of a vinylpyridine N-oxide. The exact proportion of the components can vary over a fairly wide range as long as the copolymer contains a "solubilizing quantity" of the acrylic acid ester (i.e., a sufficient quantity of acrylic acid ester to render the copolymer soluble in the lubricating oil). A preferred proportion of the components in the copolymer is from about 85 to about 97 weight percent of acrylic acid ester and from about 3 to about 15 weight percent of the vinylpyridine N-oxide, the percentages being based upon the weight of the copolymer. A more preferred proportion is from about 88 weight percent to about 94 weight percent of acrylic acid ester and from about 6 to about 12 weight percent of vinylpyridine N-oxide, the percentages being based upon weight of the copolymer.

The esters of acrylic acid employed in the formation of the novel copolymers of this invention, can be prepared by reaction of acrylic acid and an alkanol or mixture of alkanols under conventional esterification conditions. The vinylpyridine N-oxides also employed in the formation of the novel copolymers of this invention, can be prepared by the processes described in U.S. Patent 2,749,349 or other methods described in the literature.

The esters of acrylic acid contemplated are the alkyl esters thereof wherein the alkyl moieties can have up to 18 carbon atoms and preferably from 8 to 18 carbon atoms. It is desirable that at least a portion of the alkyl

2

moieties have 8 or more carbon atoms in order to promote solubility of the copolymer in the lubricating oil.

Examples of alkyl acrylates which can be employed include, among others, methyl acrylate, ethyl acrylate, propyl acrylate, isopropyl acrylate, the butyl acrylates, the pentyl acrylates, the hexyl acrylates, the heptyl acrylates, 2-ethylhexyl acrylate and other octyl acrylates, the decyl acrylates, the undecyl acrylates, the dodecyl acrylates, the tridecyl acrylates, the tetradecyl acrylates, the pentadecyl acrylates, the hexadecyl acrylates, the heptadecyl acrylates, the octadecyl acrylates, capryl acrylate, lauryl acrylate, myristyl acrylate, cetyl acrylate, stearyl acrylate, and the like. If desired, methacrylic acid may be substituted for all or part of the acrylic acid.

15 The vinylpyridine N-oxides which can be used are vinylpyridine N-oxide, lower alkyl derivatives thereof wherein preferably the alkyl group has up to 6 carbon atoms, and mixtures thereof. The vinylpyridine N-oxides contemplated can be represented by Formula I:



25 wherein R represents either hydrogen or alkyl of up to 6 carbon atoms, and wherein X represents a number having a value in the range of from 0 to 2. Preferably, the vinyl and the R groups occupy the 2 and 5 positions on the ring, which preferred embodiment can be represented by Formula II:



30 35 wherein one Y variable represents vinyl and the other Y represents either hydrogen or alkyl of up to 6 carbon atoms, and wherein X represents a number having a value of from 0 to 2. It is in general preferred that the vinylpyridine N-oxide be employed in the hydrated form, which is usually the dihydrate.

40 45 Illustrative of the vinylpyridine N-oxides which are contemplated are, among others, 2-vinylpyridine N-oxide and the dihydrate thereof, 2-methyl-5-vinylpyridine N-oxide and the dihydrate thereof, 2-vinyl-5-ethylpyridine N-oxide and the dihydrate thereof, 2-isopropyl-5-vinylpyridine N-oxide and the dihydrate thereof, 2-vinyl-5-butylpyridine N-oxide and the dihydrate thereof, 2-pentyl-5-vinylpyridine N-oxide and the dihydrate thereof, 2-hexyl-5-vinylpyridine N-oxide and the dihydrate thereof, and the like.

50 55 The copolymers employed as oil additives in the compositions of this invention may be prepared by conventional bulk, solution or dispersion methods. Preferably, the novel copolymers are prepared by reacting 70 to 97 parts by weight of an above-described ester of acrylic acid and an alkanol with 30 to 3 parts by weight of an above-described vinylpyridine N-oxide at a temperature in the range of from 20° C. to 120° C. and preferably 40° C. to 80° C. The above reaction can be carried out advantageously at pressures of up to 200 p.s.i., or more, although a range of atmospheric to 100 p.s.i. is preferred. The reaction may be conducted in the presence of, for example, 0 to 80% by weight of an inert solvent and in the presence of a polymerization catalyst. Among the solvents that may be employed are acetone, benzene, toluene, pentane, heptane and the like. Among the polymerization catalysts that may be employed are diacetyl peroxide, lauryl peroxide, isopropyl percarbonate, azobisiso-



(b) vinylpyridine N-oxide of the formula:



wherein one Y represents vinyl and the other Y represents a member of the group consisting of hydrogen and alkyl of up to 6 carbon atoms, 10 and wherein X represents a number having a value in the range of from 0 to 2, the said copolymer having a reduced viscosity in the range of from about 0.2 to about 1.5 measured in a solution of 0.2 gram of copolymer per 100 milliliters of benzene at 30° C. 15

4. The lubricating composition of claim 3 wherein said alkyl acrylate is octyl acrylate.

5. The lubricating composition of claim 3 wherein said alkyl acrylate is decyl acrylate.

6. The lubricating composition of claim 3 wherein said vinylpyridine N-oxide is 2-methyl-5-vinylpyridine N-oxide dihydrate.

References Cited in the file of this patent

UNITED STATES PATENTS

|           |               |               |
|-----------|---------------|---------------|
| 2,749,349 | Cislak        | June 5, 1956  |
| 3,030,303 | Ryan          | Apr. 17, 1962 |
| 3,058,959 | Bailey et al. | Oct. 16, 1962 |
| 3,062,824 | Dunn et al.   | Nov. 6, 1962  |